

## UNITED STATES PATENT OFFICE

1,993,600

DRAWN ARTICLE AND PROCESS OF MAKING  
THE SAME

Hugh John Fraser, Robert John Owens, Edwin Kenyon Jenckes, and John Coulter Lenhart, Huntington, W. Va., assignors to The International Nickel Company, Inc., New York, N. Y., a corporation of Delaware

No Drawing. Application February 18, 1933,  
Serial No. 657,466

21 Claims. (Cl. 205—21)

The present invention relates to drawn articles made of malleable metals or alloys and more particularly to an improved process for drawing wire, tubes, rods and the like, especially when constituted of malleable nickel-containing material, particularly alloys containing nickel and chromium.

It is an object of the present invention to provide an improved process for producing drawn articles without intermediate annealing after the various drawing operations.

It is a further object of the invention to provide a process of producing drawn articles involving an initial heat treatment in a hydrogen-containing atmosphere to impart unique characteristics to the product being drawn.

It is another object of the invention to provide an improved process for drawing wires, tubes, rods and the like which is capable of drawing the initially annealed product to its final size without subsequent annealing treatments.

It is also within the contemplation of the invention to provide a process of drawing wire which is capable of being operated in a continuous manner.

It is still a further object of the present invention to provide a method of heat treating a hot rolled rod or wire rod by annealing in a hydrogen-containing atmosphere, lead coating without pickling, and drawing the initially annealed product to its final size without subsequent annealing treatment.

Another object of the invention is to provide an improved process of drawing articles in which heavier or greater reductions per pass may be utilized, in which greater reductions of area are possible without annealing, in which greater speed of production is effected and in which pickling is eliminated.

A still further object of the invention is to provide an improved process of continuously producing drawn articles in which faster drawing speeds may be employed, in which a large portion of the handling costs are eliminated, in which only a relatively small amount of labor is required, in which a more uniform gage of product is produced, in which a decreased cost of die maintenance and replacement is effected, and in which a superior quality of finished product is obtained.

A still further object of the invention is the provision of a process of drawing products constituted of alloys of nickel and chromium which have heretofore been difficult to draw or practically impossible to draw.

Other objects and advantages of the invention will become apparent from the following description:

It has been discovered that products, particularly nickel and nickel alloys, when given a special initial heat treatment in a hydrogen containing atmosphere and then coated with lead without pickling, the product can be drawn to the final desired condition without intermediate annealing and the like. Thus, for instance, by the use of the present invention, it has been possible to draw a nickel-chromium wire rod having a diameter of about  $\frac{3}{16}$ " to a fine nickel-chromium wire having a size of about 0.001 inches. Heretofore, it has absolutely been impossible to accomplish such a procedure.

Broadly stated, the invention contemplates an initial heat treatment in a hydrogen-containing atmosphere, the temperatures ranging from about 1200° F. to about 2200° F. depending upon the constitution or the nickel content of the material under treatment. It is essential to use a reducing gas for the atmosphere which is substantially free from moisture and other oxidizing gases like carbon dioxide, and which has a relatively high concentration of hydrogen. It has been found that the hydrogen content of the atmosphere can be varied depending upon the metal or alloy under treatment and particularly the nickel content thereof.

The article which is subjected to the initial heat treatment in a hydrogen-containing atmosphere is maintained at such a temperature for a sufficient length of time to practically insure a metallic condition substantially throughout the surface skin. As yet, it has not been definitely ascertained what this special initial heat treatment in a hydrogen-containing or reducing atmosphere does to the article under treatment but it is definitely known that the metallic surface and the metal are converted into such a condition that upon direct lead coating, the article can be drawn to a fine wire or a small tube or a small rod without intermediate annealing. Results of this character have been unknown in the art and it has only been possible to draw certain nickel alloys such as nickel-chromium alloy and the like by repeated intermediate annealing and by a very complicated, cumbersome and expensive procedure. Typical of such prior procedures is one described by W. H. Wills and J. K. Findley on pages 97 to 114 in the August, 1932, issue of The Transactions of the American Society for Steel Treating. In this article the authors described the manufacture, properties and use of 18-8

30

35

40

45

50

55

chromium-nickel steel wire and discuss the necessity of annealing or heat treating the drawn or worked wire and then pickling the same in acid before further drawing or working operations can be carried out. In this connection, the authors state of chromium-nickel steel wire that:—“When subject to cold working it rapidly develops increased hardness making frequent heat treating necessary.”

After lead coating the excess of lead is removed by means of a wiper or the like. In practice, it has been found to be essential to apply the lead as a uniform layer or coating. When precautions are taken to insure the application of a uniform coat of lead, a product is produced which is substantially free from non-uniformity or variations. In passing, it might be mentioned that any appropriate procedure may be used to apply the coat of lead and to remove the excess of lead from the surface as those skilled in the art will readily understand.

The lead coated article such as a rod or the like is then subjected to a series of drawing operations. It is preferred to reduce the article in stages. In carrying the present invention into practice on an industrial scale it has been found commercially possible to make single pass reductions in area with chromium-nickel alloys of 35-40% for rods or wire and 30% for tubes which are far in excess of prior reductions. After these reductions, it is not necessary to subject the drawn article to annealing which was heretofore an indispensable operation. It has been found that repeated drawings may be employed and the article drawn to practically any desired commercial and industrial size without intermediate annealing or heat treatment.

When tubes are being drawn it has also been found that superior results can be obtained by using a rotating mandrel. The drawing of chromium-nickel tubes has been greatly facilitated by use of the rotating mandrel. Of course, conventional methods may be employed but it is preferred in carrying the present invention into practice, to employ the rotating mandrel. The mandrel is supported by appropriate means at each end thereof. At one end, the mandrel has secured thereto driving means such as a gear. This gear is connected to a prime mover, such as an electric motor by means of a suitable train of gears like a gear reducer.

After the article has been given the required number of passes to reduce the article to the desired size, it is possible to employ the article in the drawn condition. A fine film or coating of lead still remains on the surface of the wire, tube or rod and in many cases this lead film or coating is not objectionable. In those cases where it is desired to have a dealed surface, the film or coating of lead may be stripped off the surface of the article by means of an appropriate acid or the like such as a 5-10% solution of nitric acid. If desired, the dealed wire, tube or bar may be given a finishing pass or passes to impart an improved or desired surface to the article.

For the purpose of giving those skilled in the art a better understanding of the invention the following specific and illustrative examples are given:

#### Example No. 1

A hot rolled chromium-nickel alloy rod having a  $\frac{3}{4}$ " diameter and containing approximately 14% of chromium and 80 per cent of nickel was continuously annealed in a reducing atmosphere

containing hydrogen in an electrically heated furnace at about 1950° F. The thus treated wire is coated with the uniform envelope of lead in any appropriate manner. In practice, it is preferred to pass the strand of wire through a molten bath of flux which is floating upon a molten bath of lead. The wire is carried through the molten layer of lead and then out of the bath at a point which is free from flux. The lead coated wire is cooled and is then rolled into a coil. The flux may be any suitable composition but it was found that flux containing zinc chloride (8 parts by volume), sodium chloride (4 parts by volume) and ammonium chloride (1 part by volume) functions very satisfactorily and provides a surface which can be effectively lead coated. In the operation of the lead bath a temperature of about 700° F. to about 800° F. and preferably 720° F. to about 750° F. is maintained. As a result of experiments, it has been found that the lead does not have to be a pure lead but may contain impurities such as antimony, etc.

When wire is being leaded in the form of a strand, it has been found advisable to run the strand through a wiper to remove any excess of lead. In the event that the wire is leaded in coils, the latter are preferably rolled over and over in the bath to insure thorough wetting by the flux before introducing the coils into the layer of molten lead. The coils may be passed through the molten lead and then removed from the bath to permit the lead to solidify. It is preferred to throw the coils on the floor and shake them up and down until the lead has solidified, thus, preventing the strands from sticking together. In any case, it is important that the entire surface of the wire be covered with a tenaciously adhering coat of lead which is preferably as uniform as possible.

The lead coated wire is drawn through wortle dies. The amount of reduction per pass may be in excess of 35%. Thus, in the appended Table I, the passes are given with the percentage of reduction and the diameter of the wire. In addition, the breaking strength is given in pounds per square inch. In the table the elongation is given in percent per 2" and the reduction of area is given in percent.

Table No. 1

| Pass No.      | Diameter        | Percent reduction | Breaking strength | Elongation | Reduction of area | 55 |
|---------------|-----------------|-------------------|-------------------|------------|-------------------|----|
| Original..... | Inches<br>0.229 |                   | 87,000            | 45.5%      | 66.0%             |    |
| 1.....        | .162            | 50.0              | 157,000           | 6.0        | 56.4              |    |
| 2.....        | .129            | 68.3              | 173,400           | 5.0        | 43.5              |    |
| 3.....        | .095            | 82.9              | 183,500           | 3.5        | 30.4              |    |
| 4.....        | .072            | 90.0              | 207,500           | 2.5        | 33.0              |    |
| 5.....        | .057            | 93.7              | 213,000           | 2.0        | 45.7              |    |
| 6.....        | .047            | 96.0              | 212,000           | 2.0        | 45.2              |    |
| 7.....        | .035            | 97.6              | 218,000           | 1.5        | 31.4              |    |
| 8.....        | .028            | 98.4              | 241,500           |            |                   |    |
| 9.....        | .025            | 98.6              | 217,000           |            |                   |    |
| 10.....       | .022            | 98.8              | 225,000           |            |                   |    |
| 11.....       | .020            | 99.2              | 245,000           |            |                   |    |
| 12.....       | .018            | 99.3              | 246,300           |            |                   |    |
| 13.....       | .016            | 99.4              | 245,000           |            |                   |    |
| 14.....       | .014            | 99.5              | 262,000           |            |                   |    |
| 15.....       | .012            | 99.7              | 234,000           |            |                   |    |

The aforesaid alloy was not drawn smaller than .012" diameter at which point its tensile strength was greater than 200,000 psi. It could have been drawn to finer sizes.

After cold drawing, the thin coating of lead remaining on the wire was removed by dipping the wire in a 10% solution of nitric acid.

**Example No. 2**

A 1" diameter hot rolled "Monel metal" rod was bright annealed at a temperature of 1700-1750° F. in a natural gas atmosphere containing approximately 3.5 percent CO gas. The rod was then lead coated without pickling. The coated rod was drawn and Table No. 2 gives percentage of reduction, etc. for various passes.

Table No. 2

| Pass No. | Diameter | Percent reduction | Yield point | Breaking strength | Elongation | Reduction of area |
|----------|----------|-------------------|-------------|-------------------|------------|-------------------|
| 15       | Inches   |                   |             |                   |            |                   |
| Original | 1.016    |                   |             |                   |            |                   |
| 1.       | .876     | 26.0              | 30,700      | 78,200            | 62.5%      | 70.2%             |
| 2.       | .755     | 45.0              | 74,800      | 110,000           | 28.5       | 60.0              |
| 4.       | .499     | 76.2              | 93,800      | 127,500           | 22.0       | 58.0              |
| 6.       | .382     | 85.9              | 128,000     | 144,600           | 14.0       | 63.1              |
| 7.       | .314     | 90.5              | 139,000     | 153,000           | 8.0        | 52.2              |
| 8.       | .258     | 93.7              | 141,800     | 156,500           | 7.0        | 41.4              |
| 9.       | .204     | 96.1              | 153,000     | 167,100           | 5.0        | 45.6              |
| 10.      | .181     | 97.0              |             | 168,200           | 2.5        | 44.6              |
| 11.      | .143     | 98.0              |             | 171,000           | 3.0        | 61.5              |
| 12.      | .120     | 98.4              |             | 175,000           | 2.5        | 30.0              |
| 13.      | .095     | 98.8              |             | 157,200           | 2.0        | 37.4              |
| 14.      | .078     | 99.3              |             | 182,000           | 2.0        | 32.4              |
| 15.      | .061     | 99.7              |             | 185,000           | 1.5        | 30.2              |

This represents a total reduction of area of over 99.9 percent without annealing and produced a tensile strength in the wire of over 180,000 psi.

Adhering lead on the drawn wire was removed by dropping in a 10% solution of nitric acid. The wire was then washed and dried in the usual way.

**Example No. 3.**

A  $\frac{3}{8}$ " diameter hot rolled modified Elinvar (30% nickel, 62% iron and 8% chromium) wire rod was annealed in a gas fired furnace with reducing atmosphere at about 1950° F. The wire rod was then lead coated and drawn to about .140" diameter with approximately 40% reduction in area per pass.

It will be observed that the present process made it possible to make heavy reductions per pass. For comparative purposes it was found to be impossible without lead coating to draw this wire to the same degree unless it were annealed after at least every second pass. In the drawing of the wire for comparative purposes, wortle dies and soap lubricant were used in accordance with prior art practices.

For the removal of lead remaining on the wire, a 10% nitric acid solution is used.

**Example No. 4**

A  $\frac{3}{16}$ " diameter hot rolled wire rod of both Monel metal and pure nickel were annealed in a reducing atmosphere at about 1700-2000° F. and then washed in a solution containing approximately 3% tri-sodium phosphate and 7 percent soda ash. The wire was lead coated without pickling and was drawn.

The lead coated wires drew much easier and with considerable less scratching than uncoated wires and gave a superior finished product. For example, the tensile properties of the final products at .012" diameter were as follows:—

| Metals              | Breaking strength                    |
|---------------------|--------------------------------------|
| Nickel              | Over 200,000 (psi.) lbs. per sq. in. |
| "Monel metal"       | Over 200,000 (psi.) lbs. per sq. in. |
| Chrome-nickel alloy | Over 225,000 (psi.) lbs. per sq. in. |

**Example No. 5**

A chromium-nickel wire rod is annealed and lead coated as set forth in Example No. 1. The coated wire is then drawn through 4-5 wortle or metallic carbide dies successively on a continuous draw bench using 20"-24" blocks. The reductions in area are approximately 40% per pass and give wire of approximately .169", .130", .100" and .077" diameter at the successive dies.

The .077" wire is then transferred to a continuous draw bench using 12"-16" blocks and drawn through 5-6 metallic carbide dies successively, with 40-20% reductions per pass and finishing at approximately .027" diameter. As the wire becomes finer, the reduction per pass is decreased slightly. The sizes of wire at the intermediate dies on a 5 die bench are .059", .045", .036", .031" and .027" diameter.

The .027" wire is then transferred to a continuous draw bench using ten 6-8" blocks and drawn through diamond dies successively with approximately 20% reductions per pass. Metallic carbide dies may be substituted for more of the larger sizes of diamond dies. The sizes of wire at the intermediate stages on a 10 die bench are .025", .022", .020", .018", .016", .014", .0126", .011, .010 and .009" approximately. A similar procedure is used to reduce wire to sizes of .003" and smaller.

| Bench  | Speeds                    | Lubricants                               |
|--------|---------------------------|------------------------------------------|
| 20-24" | 150-1,000 ft. per min.... | Dry or wet soap, heavy lubricating oils. |
| 12-16" | 350-2,000 ft. per min.... | Dry or wet soap, heavy lubricating oils. |
| 6-8"   | 500-3,500 ft. per min.... | Wet soap or oil solutions.               |

**Example No. 6**

On the final finishing pass when drawing chromium-nickel tubes after the lead coating has been removed, scratching of the inside of the tubes is difficult and almost impossible to overcome by conventional drawing methods. It has been found that the substitution of a rotating mandrel, as noted hereinabove instead of the stationary mandrel, overcomes this drawing difficulty to a large extent and results in lower operating costs, less scrap, decreased loss of time for maintenance and repair, and a better surface quality of finished product.

It will be observed that the present invention provides a process which is capable of making total reductions greater than about 99+%.

It will also be noted that the present invention provides a process which is capable of reducing rods having a diameter of say 5" to smaller rods having a diameter of say 4" and smaller to about  $\frac{1}{2}$ ".

Furthermore, it is to be noted that the present invention provides a process for drawing wire from rods having a diameter of about 1" to wires having a smaller diameter of say  $\frac{1}{2}$ " and smaller to 0.003"-0.0005" and even to 0.001" or less without any intermediate annealing.

Moreover, it is to be observed that the present invention provides a process for drawing tubes of a variety of sizes including tubes originally having an outside diameter of  $8\frac{5}{8}$ " with a shell having a wall thickness up say about  $\frac{5}{8}$ " and that by subjecting such shells to the present procedure smaller tubes with various wall thickness can be produced by subjecting the shell to a plurality of passes say up to 12 passes or more without any intermediate annealing.

The present invention provides an improved process for the continuous or intermittent manufacture on an industrial scale of commercial cold drawn products such as rods, tubes or wire and for the manufacture of the foregoing products at faster speeds, greater reductions per pass in cold working without intermediate annealing and lower operating costs.

It will also be observed that the present invention provides a process which is especially useful in conjunction with the commercial manufacture of products made from hard alloys such as nickel alloys containing chrome, copper, manganese, aluminum, etc. which have heretofore been difficult to handle commercially and industrially because it has not been possible with prior processes to coordinate a series of heat treatments and mechanical operations and conditions and to permit continuous cold working of a product to finished size without intermediate annealing.

It will be further noted that the present invention provides a process of lead coating and drawing a hot rolled product without the customary pickling and without the necessity of usual amalgamation and without the prior intermediate annealing. With the new process a lead coating may be applied to the surface of the product under treatment and the applied lead coating will remain intact during the drawing operations and will provide a surface skin and bond with the base metal that the friction between the die and the metal being drawn is greatly reduced and the conditions are such as to permit the metal to be drawn faster with greater reductions per pass without annealing and with less scratching of the metal and of the dies and with total reductions in area of over 99% of the original size.

What is claimed is:

1. The process of manufacturing a drawn product which comprises heating a metallic product in a reducing atmosphere, enveloping the thus heated product in a leaden coat devoid of mercury amalgam and drawing the lead coated product to desired size without intermediate annealing.

2. The process of manufacturing a drawn metallic product which comprises annealing a metallic product in a reducing atmosphere substantially devoid of moisture and oxidizing gases, enveloping the thus heated product in a leaden coat without pickling, and drawing the lead coated product without annealing, said drawing being effected by reductions in excess of 35%.

3. The process of manufacturing a drawn metallic product which comprises heating a metallic product in a reducing atmosphere containing hydrogen, enveloping the thus heated product without pickling the same in a leaden coat, and drawing the product without intermediate annealing and by reductions in excess of 35%.

4. The process of manufacturing a drawn metallic product which comprises heating a metallic product in a reducing atmosphere devoid of moisture and oxidizing gases to a temperature in excess of about 1200° F. and not higher than about 2200° F. for a period of time, enveloping the thus heated metallic product without annealing the same in a substantially uniform leaden coat, and subjecting the thus coated product to a plurality of drawings without intermediate annealing, each of said drawings involving a reduction in excess of 35%.

5. The process of manufacturing a drawn metallic product which comprises heating a metallic product in a reducing atmosphere substantially

free from moisture and oxidizing gases and containing hydrogen at a temperature in excess of about 1200° F. to 2200° F. for a period of time, enveloping the thus heated product without pickling in a leaden coating, and drawing the product to desired size without intermediate annealing and by a plurality of reductions in excess of 35%.

6. The process of manufacturing a drawn metallic product which comprises passing a metallic product through a reducing atmosphere containing hydrogen, subjecting the metallic product to electrical heat at a temperature of about 1200° F. to about 2200° F. for a period of time, enveloping the thus heated product without pickling in a leaden coat, subjecting the lead coated product to a plurality of drawings without intermediate annealing, each of said drawings being in excess of 35%.

7. The process of manufacturing a drawn metallic product which comprises heating a metallic product in a reducing atmosphere containing a high concentration of hydrogen at a temperature of about 1200° F. to about 2200° F. for a period of time, applying flux to said body, enveloping the flux product in a leaden coating, and drawing the product to desired size without intermediate annealing, said drawing involving reductions in excess of 35%.

8. The process of manufacturing a drawn metallic product which comprises heating a metallic product in a reducing atmosphere substantially devoid of moisture and oxidizing gases and containing hydrogen at a temperature of about 1200° F. to 2200° F. for a period of time, applying molten flux to the heated product without pickling the same, applying a leaden coat to said fluxed product, removing excess of lead to produce a substantially uniform coat and drawing the product to desired size without intermediate annealing said drawing involving reductions in excess of 35%.

9. The process of manufacturing a drawn metallic product which comprises continuously heating a metallic product in a reducing atmosphere substantially devoid of moisture and oxidizing gases and containing hydrogen to a temperature of about 1200° F. to 2200° F. for a period of time, applying molten flux to the thus heated product without pickling the same, immersing the fluxed product in a leaden bath at a temperature of about 700° F. to 800° F., removing excess of lead from said product to produce a substantially uniform coat and continuously drawing the product without intermediate annealing, said drawing involving reductions in excess of 35%.

10. The process of manufacturing a drawn metallic product which comprises heating a metallic product in a reducing atmosphere substantially devoid of moisture and oxidizing gases and containing hydrogen at a temperature of about 1200° F. to 2200° F. for a period of time, applying molten flux to the heated product without pickling the same, applying a leaden coat to said fluxed product, removing excess of lead to produce a substantially uniform coat, drawing the product to desired size without intermediate annealing, said drawing involving reductions in excess of 35%, and subjecting the drawn product to the action of nitric acid to remove the leaden coating remaining on the surface of the product.

11. The process of manufacturing a drawn metallic product which comprises heating a metallic product containing nickel and chromium in a reducing atmosphere substantially devoid of mois-

- ture and oxidizing gases and containing hydrogen to a temperature in excess of about 1700° F. for a period of time, enveloping the heated product containing nickel and chromium without pickling the same in a substantially uniform leaden coat, and drawing the product to the desired size without intermediate annealing by the use of a plurality of reductions in excess of 35%.
12. The process of manufacturing a drawn nickel-containing product including wire, tubing and the like which comprises heating a nickel-containing product in a reducing atmosphere, enveloping the thus heated product in a leaden coat devoid of mercury amalgam, and drawing the lead coated product to desired size without intermediate annealing.
13. The process of manufacturing a drawn nickel-containing wire which comprises annealing a nickel-containing product in a reducing atmosphere substantially devoid of moisture and oxidizing gases, enveloping the thus heated product in a leaden coat without pickling, and drawing the lead coated product without annealing to produce a wire, said drawing being effected by reductions in excess of 35%.
14. The process of manufacturing a drawn nickel-chromium containing product including wire, tubing and the like which comprises heating a metallic product containing nickel and chromium in a reducing atmosphere containing hydrogen, enveloping the thus heated nickel-chromium product without pickling the same in a leaden coat, and drawing the nickel-chromium product without intermediate annealing and by reductions in excess of 35%.
15. The process of manufacturing a drawn nickel-chromium containing wire which comprises heating a metallic product containing nickel and chromium in a reducing atmosphere devoid of moisture and oxidizing gases to a temperature in excess of about 1200° F. and not higher than about 2200° F. for a period of time, enveloping the thus heated nickel-chromium containing product without annealing the same in a substantially uniform leaden coat, and subjecting the thus-coated product to a plurality of drawings without intermediate annealing to produce a nickel-chromium containing wire, each of said drawings involving a reduction in excess of 35%.
16. The process of manufacturing a drawn nickel-chromium containing product including wire, tubing and the like which comprises continuously heating a nickel-chromium containing product in a reducing atmosphere substantially devoid of moisture and oxidizing gases and containing hydrogen to a temperature of about 1200° F. to 2200° F. for a period of time, applying molten flux to the thus heated nickel-chromium containing product without pickling the same, immersing the fluxed product in a leaden bath at a temperature of about 700° F. to 800° F., removing excess of lead from said product to produce a substantially uniform coat, and continuously drawing the nickel-chromium containing product without intermediate annealing, said drawing involving reductions in excess of 35%.
17. A metallic product having a gas reduced surface covered by a lead coating and capable of being drawn without intermediate annealing.
18. A metallic product having a gas reduced surface covered by a lead coating and capable of being drawn without intermediate annealing by a plurality of reductions in excess of 35%.
19. A metallic product including wire, tubing and the like having a gas reduced surface covered by a lead coating and capable of being drawn to a wire, tubing and the like without intermediate annealing.
20. A nickel-containing product having a gas reduced surface covered by a lead coating and capable of being drawn without intermediate annealing.
21. A nickel-chromium-containing product having a gas reduced surface covered by a lead coating and capable of being drawn without intermediate annealing.

HUGH JOHN FRASER.  
ROBERT JOHN OWENS.  
EDWIN KENYON JENCKES.  
JOHN COULTER LENHART.

45